

## UNITED STATES PATENT OFFICE

2,392,646

## ELECTROPLATING TIN

William B. Cooper and Charles E. Glock, Baltimore, Md., assignors to Crown Cork & Seal Company, Inc., Baltimore, Md., a corporation of New York

No Drawing. Application July 11, 1942,  
Serial No. 450,610

## 1 Claim. (Cl. 204—54)

This invention relates to electroplating with tin and particularly to a bath for plating an indefinite length of black iron or steel strip whereby the same may be continuously passed through the plating bath and provided with a smooth uniform matte or satin finish.

The primary object of the invention is to provide an alkaline tin plating bath containing an alkali metal stannate, such as sodium stannate, and which will be stable over a wide range of operating conditions.

Another object of the invention is to provide a bath in which the sodium stannate is maintained within substantially constant critical limits and without requiring that stannate be added during plating.

A further object of the invention is to provide a sodium stannate bath in which a balance is constantly maintained between the amount of tin dissolved from the anodes and the amount deposited on the traveling strip by means of a critical alkali content whereby the tin content of the solution does not change and addition of alkali stannate during coating is made unnecessary.

An additional object of the invention is to provide a bath containing a soapy agent which will produce a foam on the surface of the plating solution, and prevent the solution from spraying, due to hydrogen being liberated at the cathode and oxygen at the anode.

Of equal importance with the foregoing, it is an object of the invention to provide an alkaline tin plating bath containing sodium stannate in which the ratio of current density of the anode to the cathode may be maintained substantially equal, i. e., 1:1, and with an anode current density of substantially 35 amperes per square foot, without requiring stannate additions during plating.

Another object of the invention is to provide an alkaline sodium stannate bath in which it is unnecessary to maintain a greenish-yellow film in order to produce smooth and uniform electro-deposited coatings of tin.

Another object of the invention is to provide a bath in which an oxidizing agent, such as hydrogen peroxide, need not be employed.

In carrying out the present invention, we will describe the same in connection with the electro-tin plating of 18 inch to 32 inch width steel strip of indefinite length. The strip is continuously traveled, first through an acid dip, then through a water rinse, then through the electroplating bath, after which it is spray-washed and dried.

The operations are carried out in a "line," and the strip never stops during the various operations, due to the use of loopers so situated that the ends of the coils of strip can be welded together and the finished coated coils stripped while the band is in continuous motion.

By strip steel, we mean various grades available and useful for the manufacture of containers and container closures, among which may be mentioned low carbon rimmed steel, low carbon killed steel, and rephosphorized steel, as well as ordinary black iron strip. The strip is of the usual thicknesses employed for making containers and closure caps of sheet metal.

15 The pickling operation on the traveling strip is preferably carried out in a sulfuric acid solution of 3 to 6%  $H_2SO_4$  by weight in water at 170° F., using an inhibitor to prohibit etching of the strip. The sheet as it leaves the acid tank is covered by a film of acid since otherwise, a superficial oxide will form on its surface and the subsequent tinning will be marred.

20 The traveling strip is then rinsed free of acid in a simple dip tank having clean water constantly replacing the acid contaminated water resulting from the carry over of acid. The tank is baffled so that fresh water enters as the sheet leaves and is drained off at the entry side. The rinse water is removed from the sheet as close

25 to the plating bath as is practical. This is done to eliminate the superficial oxidation that will result whenever the sheet is exposed for a short time to the atmosphere. The faster the strip travels, the less trouble is experienced with this type of oxidation. A squeegee roll is employed to remove most of the rinse water and so constructed that a residual, continuous film of water remains on the sheet whereby the strip is protected until immersion in the plating solution to which

30 it now passed.

A preferred plating solution found to give consistently good results has substantially the following formula:

35 Tin (as sodium stannate) ----- Substantially 30/45 g./l.  
Sodium hydroxide ----- Substantially 10/12 g./l.  
Hydrogen peroxide (optional) ----- Substantially  $\frac{1}{4}$  pt. every  $\frac{1}{2}$  hr. to 10,500 gallon tank.  
Ridosol #14 ----- Substantially sufficient amount to obtain a blanket of foam. 1 qt. to 10,500 gallons of plating solution.

40 Temperature ----- About 190° F.

The plating tank has a capacity of about 10,500 gallons, and the tin anodes are disposed vertically therein in spaced relation. The traveling

strip is coated while traveling parallel to the anode surfaces in the above bath.

When the caustic content is allowed to go as low as 9 g./l. (as NaOH), excessive sludging of the bath results, and if raised above 16 g./l., a good smooth coating cannot be obtained. When the tin content drops below 30 g./l., the plating becomes very dull and loses its satin or matte appearance. As the tin content goes above 45 g./l., tin tends to deposit on the current carrying rolls, forming objectionable "tin pimples." These put small dents in the strip and must be scraped from the rolls.

We have discovered that if the caustic content is kept within the critical limits described, a balance is maintained between the amount of tin dissolved from the anodes and the amount deposited on the traveling strip. In this manner, the tin content of the solution does not change, as demonstrated by the fact that no additions of sodium stannate were necessary over a several-month period with a line operating at speeds up to 370 ft./min. on 29" wide material 24 hours a day and seven days a week. An anode current density of 35 amp./sq. ft. is used in normal operation, and the anode to cathode ratio is roughly 1:1. This current density allows the anode to corrode uniformly, and no special treatment is necessary to maintain the anodes in good condition.

"Ridosol" #14 is an agent which is of soapy character and is added to the alkaline tin plating bath to produce a foam on the surface of the plating solution. This foam prevents the solution from spraying, which is caused by hydrogen being liberated at the cathode and oxygen at the anode. These gases, rising out of the solution as very fine bubbles, carry some of the caustic plating solution with them and thereby causes discomfort to the people working in the vicinity. In addition, parts of the nearby machinery are coated with this caustic compound. The foam collects these gases and subsequently releases them in larger masses and at a slower velocity.

The "Ridosol" also reduces the surface tension of the solution, thus increasing its detergent properties. The solution has a greater tendency to plate more uniformly even on fairly greasy surfaces.

If desired, sodium acetate can be used in the bath but is not necessary after the bath has been in operation for a time. Its primary action seems to be in buffering the solution.

In order to eliminate the use of hydrogen peroxide, we employ one iron anode 15" wide by 88" long, which appears to guard against formation of spongy deposits.

There are 31 pure tin anodes which will supply the bath with sufficient tin to maintain the proper tin content, each anode having a dimension of substantially 32" wide by 89" long. All of the anode is not immersed in the solution. The part immersed is 77" by 32".

If desired, sodium cyanide may be added to the bath for promoting anode corrosion. It is beneficial in obtaining a good satin finish, and where the satin finish tin plate is subjected to brightening as by a fusing operation, the brightening appears to be facilitated. Sodium cyanide is not preferred due to its creation of a health hazard.

Sodium orthosilicate in amount of about up to 13 grams per liter may be used to replace caustic soda with good results when the bath is fresh, but on aging for a few days, a silicious precipitate forms. This precipitate can be redissolved

by additions of caustic soda. This bath is not considered to be as practical in operation as one using caustic. By way of example, the composition of an orthosilicate bath is:

5 Tin (as sodium stannate) ..... g./l. 30  
Sodium orthosilicate ..... g./l. 13  
Sodium acetate ..... g./l. 10

Sodium phosphate to replace sodium hydroxide 10 may be added to the stannate bath in amount of up to about 25 g./l. and a good plating obtained.

Also, an alkaline bath made up of sodium sulfide replacing sodium hydroxide and sodium stannate as the principal constituents will produce 15 satisfactory tin plating. An example of the composition of a sodium sulfide bath is:

Tin (as sodium stannate) ..... g./l. 50  
Sodium sulfide (Na<sub>2</sub>S) ..... g./l. 15

The solution was filtered and operated at 170° F. giving very good results.

Sodium orthosilicate, sodium phosphate and sodium sulfide have all been used to replace sodium hydroxide, all or in part.

In the use of the alkali, such as the caustic or the equivalent alkaline materials, the amount present in the bath is always effective to maintain a constant balance between the quantities of anode dissolved tin and deposited tin, whereby plating on a strip of indefinite length may be carried out continuously without necessity of adding stannate to the bath during the coating.

The strip leaves the plating tank through two sets of wringer rolls. The first set removes most 35 of the plating solution. The second set is supplied with water sprays which wash most of the remainder of the solution back into the plating tank. A balance is maintained between the rinse water entering the tank and water lost by evaporation 40 so that the amount of solution is constant. The solution is constantly filtered to remove any coarser particles.

The coated strip, after leaving the plating bath, is subjected to high pressure hot water sprays in a rinse tank. These sprays thoroughly clean the 45 strip without scratching or otherwise changing the surface of the coating. It then passes through wringer rolls to a drying tunnel consisting of a blast of hot air and then the strip is continuously coiled and is ready for the next 50 operation. This step can consist of shearing to sheets or a reflowing or brightening operation by fusing the tin surface or cold rolling.

A tabulation of line speed and coating weights 55 is here shown for illustrating the advantageous results obtained by employing the critical ranges of caustic and stannate specified:

[Speed vs. coating on 29" wide (average) strip]

| Ft./min. | Amperage | Solution composition |           | Tin coating |
|----------|----------|----------------------|-----------|-------------|
|          |          | G. Sn/l              | G. NaOH/l |             |
| 65       | 40,000   | 42.41                | 10.51     | .32         |
| 290      | 40,000   | 38.94                | 10.03     | .40         |
| 250      | 40,000   | 36.94                | 10.12     | .50         |
| 210      | 40,000   | 39.52                | 11.11     | .58         |
| 195      | 40,000   | 39.27                | 11.35     | .70         |
| 160      | 40,000   | 40.22                | 10.95     | .75         |
| 150      | 40,000   | 38.70                | 10.03     | .81         |

70 While we have referred herein to continuous strip metal as being successfully coated, it is to be understood that other continuous materials, such as wire, as well as individual objects, are

susceptible of being electroplated with equally satisfactory results.

Rodosol #14 is a product the composition of which usually is of complex organic nature, that is, sulphonated hydrocarbons. It is of a soap forming material and can be replaced by soaps such as sodium palmitate, oleate, etc.

We claim:

A process for the electrodeposition of metallic tin comprising conducting an electrolyzing current from a tin anode to the article to be coated as a cathode through an aqueous solution having a temperature of about 190° F. and comprising

5 ing essentially sodium stannate to give substantially 30 to 45 grams per liter of tin and sodium hydroxide substantially 10 to 12 grams per liter to produce a substantially constant balance between the quantities of anode dissolved tin and deposited tin, maintaining an anode current density of substantially thirty five amperes per square foot with a ratio of current densities of anode to cathode of substantially 1:1 and an anode to cathode ratio of about 1:1.

10 WILLIAM B. COOPER.  
CHARLES E. GLOCK.